

## UNITED STATES PATENT OFFICE

ALFRED HENRIKSEN, OF PONCA CITY, OKLAHOMA, ASSIGNOR TO CONTINENTAL OIL COMPANY, OF PONCA CITY, OKLAHOMA, A CORPORATION OF DELAWARE

## METHOD OF DEWAXING OILS

No Drawing.

Application filed January 18, 1930. Serial No. 421,815.

This invention relates to the treatment of petroleum oils and refers particularly to the method of purifying lubricating oils by the use of colloidal wax adhering substances in 5 a continuous centrifuge process.

In the production of lubricating oils, one of the troublesome group of compounds encountered is the waxes. These waxes vary from low melting point amorphous wax to 10 high melting crystalline wax and are compounds of the paraffin series. Lubricating oils to be used at low temperatures must have these waxes removed in order to obtain free movement of the lubricating medium; moreover, the waxes themselves are of 15 very poor lubricating value and act as a detriment to the lubricating qualities of the oil. High wax content oils, being solid at relatively high temperatures, give considerable trouble in refining practice because 20 they cannot be pumped or require heated tanks for cold weather storage.

Oil refiners have developed three general methods of wax separation:

- 25 1. Lubricating stock dilution with naphtha, chilling and pressing.
2. Lubricating stock dilution with naphtha, chilling and cold settling.
3. Lubricating stock dilution with naphtha, chilling and centrifuging.

These general methods have taken on various modifications in an effort to solve the dewaxing problem.

A brief outline of the refinery practice on 35 paraffin base crudes will show the essentials of wax separation methods. The ordinary break-up of crude in the refinery is: 1, naphtha; 2, kerosene; 3, gas oil; 4, wax distillate; 5, residue-steam refined cylinder stock. The naphtha, kerosene and gas oil are removed by distillation, every processing detail being guarded to obtain the residue in as good condition as possible. Still 40 temperature, rate of distillation, amount of steam, etc. are regulated to prevent injury of the residue. The wax distillate is removed at as low still temperature as possible, using large amounts of steam. This 45 gives the crystalline waxes in the overhead

wax distillate and the amorphous waxes in the residue.

The amount of crystalline-amorphous wax separation depends on the nature of the crude and control of the refining process. The wax distillate is either chilled and 55 pressed directly or given a heating treatment with a small amount of steam, called "cracking wax distillate," then chilled and cold pressed.

The steam refined cylinder stock requires other treatment to obtain high class lubricating oil price. This further refining includes acid treating and/or clay treating, 60 which treating causes the waxes to be less soluble and a higher pour point results on the finished stock. For example, a steam refined stock may have a 40° F. pour point before treating with acid and/or clay for color and removal of impurities, and an 80° F. 65 pour point after treatment.

It is, therefore, necessary to dewax the finished oil. If the stock is diluted with naphtha and chilled, the wax crystals will 70 form and settle to the bottom of the container. This is a very slow process requiring several days for completion, and gives a rather poor separation and a large loss of stock in the settled wax solvent solution.

The chilling is done slowly at the top of the 75 container and the wax crystals start flowing to the bottom, care being taken that no external agitation is obtained; therefore, the process could not be continuous. This process may be more successfully operated if a 80 heavy finely divided substance, that is wax adherent, is added to give a greater gravity difference between the oil and the wax. With wax settling conditions, high investment in plant equipment is required; high 85 operating costs for long time refrigeration is involved; large volumes of oil are tied up in the process and maximum yields of high class cylinder stocks cannot be obtained. Many types of stocks contain wax 90 which cannot be separated by this method.

Others have invented processes of wax separation which consists of naphtha dilution, the addition of clay and finely divided 95 solids, chilling, and filter pressing. On 100

chilling, the wax separates from the oil and is held by the finely divided solid material suspended in the oil; also the finely divided material forms a mat with the wax and aids in holding the wax from passing through the filter cloth. After the filter has been in operation for a short period, the finely divided solid and wax form such a thick bed on the filter cloth that the process must be stopped and the filter cloth cleaned. This process is a batch process and the regular required cleaning of the filter cloth is costly and cuts down the unit volume throughput. To process an oil by this method, the wax must be in a specific form. Some oils will not give up their wax by this process.

When a lubricating stock is diluted with naphtha and chilled, the wax crystals that separate out have a slightly higher specific gravity than the solvent oil mixture. Advantage is taken of this characteristic in wax removal by high speed centrifuge. The wax bodies are thrown out by the centrifugal action into the outer compartment of a special apparatus from which they are removed by a warmer solution. The partly dewaxed lube oil stock—naphtha solution passes on up and out of the centrifuge. The density of the wax is so near that of the mother liquor that separation of wax is rather poor. Under the best operating conditions, one obtains a pour point on the finished oil of about 35° F to 40° F. higher than the temperature at which the solution goes to the centrifuge.

To dewax stocks with the centrifuge, they must be very carefully blended to the proper gravity with the solvent used. Another disadvantage of this process is the time and required regularity of cooling. After the careful blending, the solution must be chilled at a slow rate requiring, as a rule, nearly twenty four hours for chilling; the chilling rate usually is from 3° F. to 6° F. per hour, depending on the stock, solvent and result required.

Some stocks cannot be dewaxed by the centrifuge process, even though all known disturbing factors are controlled.

The present invention provides an improved method of separation of wax from cold type stock mixtures, or from crude petrodatum stock produced by present dewaxing methods, or from other fractions from which separation of wax is desired. Objects of the present invention are:

1. More nearly complete wax separation by centrifugal action.
2. Wax removal in centrifuge with the aid of colloidal substances in the stock naphtha solution.
3. Continuous wax removal in the centrifuge by the addition of centrifuge aids.
4. Continuous wax removal in the cen-

trifuge by the addition of bituminous colloidal centrifuge aids.

5. Centrifugal continuous wax removal using substances capable of forming a dispersoid in the solvent used.

6. Wax removal which allows the shock-chilling of the stock naptha solution without the detrimental effects obtained in other methods by shock-chilling.

In the operation of this method, the stock to be dewaxed is diluted with a suitable solvent, such as naphtha, any of the heavy alcohols, benzol, acetone and similar organic solvents, or any other solvent which will give a wax-solution density differential, and remain liquid at the temperatures used. To this solution is added a substance which will give a colloidal solution. Such substances as bitumen, Grahamite and the like, which are not soluble or are only partly soluble in the solution, are desirable. This material may be added before chilling, during chilling, or after the chilling period. In actual practice the most satisfactory method for adding the centrifuging aid to the oil to be treated is to prepare the colloidal solution of the centrifuging aid in a suitable medium and add the colloidal solution at any point in the chilling process prior to centrifuging. The solvent in which the colloidal solute is converted to a colloidal solution may be the same or different from the diluent used for the oil.

The chilled stock-naphtha blend with the centrifuge aid added is now charged to the centrifuge where the wax and centrifuge aid are easily thrown out of the oil naphtha solution. The nature of the centrifuge aid allows it to be easily washed out of the centrifuge with the wax without obstructing or clogging the system. This advantage is not present in finely divided or inorganic pulverized solids which would not flow from a high speed centrifuge. As in other centrifugal processes, the de-waxed stock-solvent solution is drawn off the top of the centrifuge from which the de-waxed lubricating stock is recovered.

In presenting this invention the term bitumen is used to include that class of substances consisting mainly of hydrocarbons and including the hard, solid, brittle varieties called asphalt, the semi-solid maltha and mineral tars. The term bitumen as used herein also includes the substances that are removed with sulfuric acid and/or clay treating as/or with coloring matter and acid soluble constituents; maltha being the class of substances intermediate between asphalt and petroleum.

The definition of the term centrifuge-aid is apparent from the context of the specification.

The term centrifuge-aid is used to include substances which allow better operation of the centrifuge, substances which in any way

alter the nature of the wax particles and assist the centrifuge in their efficient separation from the stock-solvent solution, substances which alter the nature of the solvent and cause the wax to be less soluble or more easily precipitated at the temperatures and dilutions used.

In the application of the process many comparisons of the merits of our process 10 and the other type processes have been made. For example, two stocks can be chosen, one of which may be de-waxed at the centrifuge and not de-waxed by the cold pressing with filter-aid process; the other 15 being de-waxed by the cold pressing with a filter-aid process and not de-waxed at the centrifuge. By conditioning these two stocks for my process, that is, by adding a centrifuge-aid, I can de-wax both at the 20 centrifuge.

Numerous colloidal agents have been found that have given satisfactory commercial results. In the practice of this process it has been found that the centrifuge-aid required for de-waxing one stock 25 may be found in another stock which is to be de-waxed and in such cases the centrifuge-aid naturally existing in one stock may be utilized by blending with the other.

30 The material or centrifuge-aid thought to be bitumen or the constituents thereof may be:

(a) Naturally present in the oil or its residues to be processed;

35 (b) Present in excess of requirement in one stock and deficient in another, so blended will give proper percentage;

(c) A product of addition.

An example of (a) is as follows:

40 A cylinder stock produced from Tonkawa crude after acid treating and neutralizing was dissolved or blended in the proportion of 2 parts naphtha to 1 part oil, chilled to minus 15° F. and centrifuged, giving good 45 wax separation and a finished oil having pour test of 15° F. The above indicates that oil from this source contains at least sufficient centrifuge-aid to give satisfactory wax separation.

50 An example of (b) is a cylinder stock made by distillation overhead from dark colored average Mid-Continent crude, when acid treated, neutralized and dissolved in naphtha and chilled to minus 15° F. as 55 above, gives unsatisfactory wax separation with a resulting pour test on the finished oil of from 70° F. to 100° F. When 2 parts of this overhead distillate Mid-Continent oil was blended with 3 parts of the Tonkawa

60 cylinder stock or flux from this cylinder stock in smaller quantities mentioned under (a) and the mixture blended, chilled and centrifuged as above, there was a satisfactory wax separation with a resulting pour test on the finished oil of 20° F. A residue,

flux or extract from distillation of some oils contain the centrifuge aid contemplated herein.

The following examples, which include examples of (c), are not to be considered a limitation of the invention, it being understood that these are just a few examples given to make clear the operation of the process. Some of the examples also disclose the use of a bitumen in combination 75 with petrolatum.

#### Example 1

Overhead lube treated with 30# 95% sulfuric acid per barrel and 15% clay showing on the treated oil

| Gravity | Viscosity | Pour point |
|---------|-----------|------------|
| 24.2    | 87        | 105° F.    |

85

this treated stock was added to 65.1% of a 55.7° Bé. gravity naphtha and chilled at 6° F. per hour to -15° F. The wax under these conditions could not be separated by 90 centrifuging but with the addition of .1% bitumen and passing through centrifuge, a pour point of 20° F. was obtained. Petrolatum alone does not give as efficient wax removal on this crude as petrolatum blended 95 with bitumen.

#### Example 2

A treated overhead lube stock of the following character:

| Gr.  | Fl.     | Fr.     | Vis. | Pour pt. | Color          |
|------|---------|---------|------|----------|----------------|
| 23.7 | 490° F. | 565° F. | 80   | 100° F.  | 2-Tag.Robinson |

100

was blended with 68.5% of 57.4 gravity 105 naphtha, to which was added 0.025% California bitumen and 2% petrolatum. This was chilled at 6° F. per hour to minus 40° F. and gave at the centrifuge after finishing a lubricating stock of pour point 8° F., filtered through clay 200 bbls/ton.

| Gr.  | Fl. | Fr. | Vis. | Pour point | Color      |
|------|-----|-----|------|------------|------------|
| 22.0 | 500 | 580 | 90   | 7° F.      | 1 1/4 T.R. |

110

#### Example 3

A commercial product known as Grahamite to an amount of 0.1% was used with success lowering the pour point on the 120 finished oil 50° F. By use of 0.1% Grahamite and 2% petrolatum, the pour point was lowered on the finished stock 65° F.

#### Example 4

A treated overhead lube stock was diluted, chilled and centrifuged yielding a finished stock of 44° F. pour point. The centrifuged stock was blended with 56.9% of 54.6 gravity naphtha and 0.2% Montan wax, chilled at 130

6° F. per hour to -15° F.; then centrifuged yielding a finished product of 25° F. pour point; operating same as above with the addition of 0.05% bitumen gave a 5 finished product of 15° F. pour point.

By extensive actual tests, I have found that any bituminous substance that is not soluble or partly soluble at centrifuging temperatures used proves satisfactory in the 10 operation of this process. I have further found that substances which give a dispersoid solution of naptha and lubricating oil proves satisfactory. I believe that the dispersoid gives a nucleus around which the 15 wax gathers, forming a body of greater density than the solution from which the wax came. The centrifuge can then make a better separation. It is to be clearly understood that this patent is independent 20 of any theory offered.

I claim as my invention:

1. A method for removing wax from wax-containing oils comprising the steps of adding a suitable solvent and a colloidal asphaltite, chilling the mixture to the desired temperature, and subjecting the chilled mixture 25 to a centrifugal action.

2. A method for removing wax from wax-containing oils comprising the steps of adding a suitable solvent and Grahamite, chilling the mixture to the desired temperature and subjecting the chilled mixture to a centrifugal action.

3. A method for removing wax from wax-containing oils comprising the steps of adding a suitable solvent and a mixture of Grahamite and petrolatum, chilling the resulting mixture to the desired temperature, and subjecting the chilled mixture to a centrifugal action.

40 4. A method for removing wax from wax-containing oils comprising the steps of adding a suitable solvent and on asphaltite capable of forming a dispersoid in the solution, chilling the mixture to the desired temperature and subjecting the chilled oil to 45 a centrifugal action.

In testimony whereof I affix my signature.

ALFRED HENRIKSEN.